

# UNITED STATES PATENT OFFICE.

WILLIAM SONDERGARD, OF SPOKANE, WASHINGTON.

COMPOSITION OF MATTER TO BE USED BY SHOW-CARD WRITERS, ARTISTS, AND ARCHITECTS, FOR PEN, BRUSH, AND AIR-BRUSH WORK.

1,358,996.

Specification of Letters Patent. Patented Nov. 16, 1920.

No Drawing.

Application filed February 7, 1920. Serial No. 357.034.

To all whom it may concern:

Be it known that I, WILLIAM SONDERGARD, a Canadian subject, and a resident of the city of Spokane, Spokane county, State of Washington, have invented a new and useful Improvement in a Composition of Matter to be Used by Show-Card Writers, Artists, and Architects, for Pen, Brush, and Air-Brush Work, of which the following is a specification.

I use 1 oz. of striping or lining bronze, which are very finely ground impalpable metallic powders. My reason for using them being, that they are ground much finer than other powders.

I add to the bronze  $\frac{1}{2}$  oz. of mucilaginous adhesive and 1 oz. of water. When thoroughly mixed, leave over night, then skim well without disturbing settling. After skimming stir up composition. Leave stand a few hours, repeat skimming three or four times until no scum rises to the top. This scum has its origin in the powder, and consists of very fine particles of the powder that have not been thoroughly mixed with the adhesive, when water was added. It is then ready for brush and can be thinned further with water for pen or air brush work.

A great want has long been and now is felt for a gold and silver watercolor that will "cover" and look smooth and that can be used with an air brush.

There are at present water colors on the market. These are made of coarser powders than I use. They will not cover with a brush and cannot be used for air brush work.

My composition is intended to be an improvement over existing makes in that it is made of only the very finest ground powders and a thin mucilaginous adhesive, a combination which allows it to pass through the small air brush and which also makes it cover well and enables the show card writers to use it for either pen or brush work with satisfactory results.

Striping or lining bronzes, these being the very finest ground metallic powders, have been or now are used with a mucilaginous adhesive.

What I claim and desire to secure by Letters Patent of the United States is:

A composition of finest ground metallic powders and a mucilaginous adhesive.

In testimony that I claim the foregoing as my invention or improvement, I have signed my name in presence of two witnesses, this 2nd day of February, 1920.

WILLIAM SONDERGARD.

Witnesses:

F. J. CURTIS,  
H. L. ECOWAN.